



US011865410B1

(12) **United States Patent**  
**Chavan**

(10) **Patent No.:** US 11,865,410 B1  
(45) **Date of Patent:** Jan. 9, 2024

(54) **GOLF BALL WITH AN ACID-FUNCTIONAL POLYURETHANE HYBRID**

(71) Applicant: **Callaway Golf Company**, Carlsbad, CA (US)

(72) Inventor: **Vijay Chavan**, Vista, CA (US)

(73) Assignee: **Topgolf Callaway Brands Corp.**, Carlsbad, CA (US)

(\*) Notice: Subject to any disclaimer, the term of this patent is extended or adjusted under 35 U.S.C. 154(b) by 0 days.

(21) Appl. No.: **17/380,980**

(22) Filed: **Jul. 20, 2021**

**Related U.S. Application Data**

(60) Provisional application No. 63/055,505, filed on Jul. 23, 2020.

(51) **Int. Cl.**

*A63B 37/06* (2006.01)  
*A63B 37/00* (2006.01)

(52) **U.S. Cl.**

CPC ..... *A63B 37/0076* (2013.01); *A63B 37/0059* (2013.01); *A63B 37/00621* (2020.08)

(58) **Field of Classification Search**

CPC ..... A63B 37/0023; A63B 37/0038; A63B 37/0072

USPC ..... 473/376

See application file for complete search history.

(56) **References Cited**

**U.S. PATENT DOCUMENTS**

2006/0189733 A1\* 8/2006 Kennedy, III ..... A63B 37/0075 525/88

2018/0085635 A1\* 3/2018 Chavan ..... C01B 32/182

2019/0217157 A1\* 7/2019 Sullivan ..... C08G 18/3893

\* cited by examiner

*Primary Examiner* — Raeann Gorden

(74) *Attorney, Agent, or Firm* — Michael A. Catania

(57) **ABSTRACT**

A golf ball with a cover or mantle layer that comprises a polyurethane and ionomer hybrid made by compounding or dry blending acid functional polyurethane and an ionomer is disclosed herein. The golf ball comprises a core (single core or dual core), a mantle layer (single layer or dual layer) and a cover layer.

**9 Claims, 13 Drawing Sheets**





FIG. 1



FIG. 2



FIG. 3



FIG. 4



FIG. 5



FIG. 5A



FIG. 6



FIG. 7



FIG. 8



FIG. 9



FIG. 10



FIG. 11



FIG. 12



FIG. 13



FIG. 14



FIG. 15



FIG. 16



FIG. 17



FIG. 18



FIG. 19

## GOLF BALL WITH AN ACID-FUNCTIONAL POLYURETHANE HYBRID

### CROSS REFERENCES TO RELATED APPLICATIONS

The Present Application claims priority to U.S. Provisional Patent Application Number 63/055,505, filed on Jul. 23, 2020, which is hereby incorporated by reference in its entirety.

### STATEMENT REGARDING FEDERALLY SPONSORED

### RESEARCH OR DEVELOPMENT

Not Applicable

### BACKGROUND OF THE INVENTION

### FIELD OF THE INVENTION

The present invention generally relates to a golf ball with a layer incorporating an acid-functional polyurethane hybrid.

### DESCRIPTION OF THE RELATED ART

Since its discovery in 2004, graphene has attracted tremendous academic as well as industrial interest. It is 100 times stronger than steel, 50% electrically and 10 times thermally more conductive than copper. It also has one of the best-known gas barrier properties. Recently due to advances in its manufacturing process, cost of graphene has come down significantly. This reduced cost combined with its superior properties has resulted in many successful commercial products.

### BRIEF SUMMARY OF THE INVENTION

The primary objective of this invention is to alter the physical properties and spin profile of a golf ball by incorporation of a polyurethane and ionomer hybrid material for use in a cover or mantle layer of the golf ball.

One aspect of the present invention is a golf ball comprising a center core, a mantle layer and a cover layer disposed over the mantle layer. At least one of the cover layer or the mantle layer comprises a polyurethane and ionomer hybrid made by compounding or dry blending acid functional polyurethane and ionomer.

Another aspect of the present invention is a golf ball comprising a dual core comprising an inner core and an outer disposed over the inner core, a mantle layer disposed over the inner core, and a cover layer disposed over the mantle layer. At least one of the cover layer or the mantle layer comprises a polyurethane and ionomer hybrid made by compounding or dry blending acid functional polyurethane and ionomer.

Yet another aspect of the present invention is a golf ball comprising a core, an inner mantle layer disposed over the core, an outer mantle layer disposed over the inner mantle layer, and a cover layer disposed over the outer mantle layer. At least one of the cover layer, the inner mantle layer or the outer mantle layer comprises a polyurethane and ionomer hybrid made by compounding or dry blending acid functional polyurethane and ionomer.

Having briefly described the present invention, the above and further objects, features and advantages thereof will be recognized by those skilled in the pertinent art from the following detailed description of the invention when taken in conjunction with the accompanying drawings.

### BRIEF DESCRIPTION OF THE SEVERAL VIEWS OF THE DRAWINGS

- 10 FIG. 1 is a partial cut-away view of a golf ball.  
 FIG. 2 is top perspective view of a golf ball.  
 FIG. 3 is a cross-sectional view of a core component of a golf ball.  
 FIG. 4 is a cross-sectional view of a core component and a mantle component of a golf ball.  
 15 FIG. 5 is a cross-sectional view of an inner core layer, an outer core layer, an inner mantle layer, an outer mantle layer and a cover layer of a golf ball.  
 FIG. 5A is a cross-sectional view of an inner core layer, an intermediate core layer, an outer core layer, a mantle layer and a cover layer of a golf ball.  
 20 FIG. 6 is a cross-sectional view of an inner core layer under a 100 kilogram load.  
 FIG. 7 is a cross-sectional view of a core under a 100 kilogram load.  
 25 FIG. 8 is a cross-sectional view of a core component and a mantle component of a golf ball.  
 FIG. 9 is a cross-sectional view of a core component, the mantle component and a cover layer of a golf ball.  
 FIG. 10 is a partial cut-away view of a four-piece golf ball.  
 FIG. 11 is a partial cut-away view of a three-piece golf ball.  
 30 FIG. 12 is a partial cut-away view of a two-piece golf ball.  
 FIG. 13 is a cross-sectional view of a two-piece golf ball.  
 FIG. 14 is a cross-sectional view of a three-piece golf ball.  
 FIG. 15 is a partial cut-away view of a three-piece golf ball.  
 FIG. 16 is a cross-sectional view of a three-piece golf ball with a dual core and a cover.  
 35 FIG. 17 is a cross-sectional view of a three-piece golf ball with a core, mantle and cover.  
 FIG. 18 is a cross-sectional view of a four-piece golf ball with a dual core, mantle layer and a cover.  
 40 FIG. 19 is a cross-sectional view of a four-piece golf ball with a core, an inner mantle layer, an outer mantle layer, and a cover.

### DETAILED DESCRIPTION OF THE INVENTION

The present invention is preferably a golf ball cover layer or mantle layer having acid-functional polyurethane hybrid material.

55 Polyurethane and ionomer hybrid made by compounding or dry blending acid functional polyurethane and ionomer.

The acid functional polyurethane is preferably made by reacting an isocyanate functional polymer with molecules that have both hydroxyl and acid functionalities. They preferably have one or more hydroxyl and one or more acid functional groups present on them. A weight percent of the molecules in the polyurethane range between 0.5 to 70 of the polyurethane.

60 The polymer is optionally neutralized with various salts that include but are not limited to sodium carbonate, sodium hydroxide, magnesium oxide, magnesium hydroxide, zinc oxide, zinc hydroxide, zirconium oxide, zirconium hydrox-

ide, titanium dioxide, potassium carbonate, lithium carbonate, calcium oxide, calcium hydroxide before blending or compounding with ionomer. Monomers used for making ionomers described in this invention include but are not limited to ethylene, propylene, methacrylic acid, acrylic acid, n-butyl acrylate, methyl methacrylate. Acid groups present on these ionomers may be neutralized by salts/bases of one or more of following cations: sodium, potassium, magnesium, zinc, zirconium, titanium, lithium, calcium.

Optionally maleic anhydride functional polymers is added to such hybrid polymer. A base resin of such functional polymers is made from fully or partially hydrogenated styrene butadiene or styrene isoprene.

This hybrid polymer can be used in mantles or cover of golf balls.

Physical properties and spin profile of a golf ball is changed by incorporation of polyurethane and ionomer hybrid.

Four different single cores (formula 1 to 4) were made as shown in recipe in Table 1. Control group (formula 1) had no graphene

already molded inner core having a diameter of approximately 0.940" and a soft compression of approximately 0.200 inches of deflection under a 200 lb load. Curing of the inner and outer core was done at temperatures ranging between 150-400° F. for times ranging from 1-30 minutes. After molding, the dual cores were spherically ground to approximately 1.554" prior to testing.

Table 2 and 3 give details of recipe of inner and outer cores. Components from these recipes were mixed in an internal mixer. Optionally, additional mixing was done using a two roll mill.

Compression of the outer core is measured by first making a full size core separately, measuring its compression, and then molding two halves around the inner core to complete the dual core.

Compression differential describes the difference between the outer core compression (as molded independently) and inner core compression. A higher compression differential is more susceptible to crack durability upon impact.

TABLE 1

| Components                                                                                         | Recipe of solid core (graphene)  |                                    |                                    |                                    |
|----------------------------------------------------------------------------------------------------|----------------------------------|------------------------------------|------------------------------------|------------------------------------|
|                                                                                                    | Formula 1<br>(0%)<br>Graphene A) | Formula 2<br>(0.4%)<br>Graphene A) | Formula 3<br>(0.8%)<br>Graphene A) | Formula 4<br>(1.6%)<br>Graphene A) |
|                                                                                                    | % wt                             | % wt                               | % wt                               | % wt                               |
| Polybutadiene                                                                                      | 62.5                             | 62.3                               | 62.1                               | 61.5                               |
| Zinc Diacrylate                                                                                    | 19.9                             | 19.8                               | 19.7                               | 19.6                               |
| Zinc Oxide                                                                                         | 6.3                              | 6.2                                | 6.2                                | 6.2                                |
| Zinc Stearate                                                                                      | 3.8                              | 3.7                                | 3.7                                | 3.7                                |
| Peroxide initiator                                                                                 | 0.5                              | 0.5                                | 0.5                                | 0.5                                |
| Zinc pentachlorothiophenol                                                                         | 0.6                              | 0.6                                | 0.6                                | 0.6                                |
| Color                                                                                              | 0.1                              | 0.1                                | 0.1                                | 0.1                                |
| Limestone                                                                                          | 0.0                              | 0.0                                | 0.0                                | 0.0                                |
| Tungsten                                                                                           | 0.0                              | 0.0                                | 0.0                                | 0.0                                |
| Barium sulfate                                                                                     | 6.4                              | 6.4                                | 6.4                                | 6.3                                |
| Graphene A                                                                                         | 0.0                              | 0.4                                | 0.8                                | 1.6                                |
| Graphene A in masterbatch                                                                          | 0.0                              | 0.0                                | 0.0                                | 0.0                                |
| Properties of core                                                                                 |                                  |                                    |                                    |                                    |
| Compression                                                                                        | 69.4                             | 74.3                               | 74.6                               | 76.4                               |
| COR (coefficient of restitution @ 125 fps)                                                         | 0.801                            | 0.800                              | 0.795                              | 0.790                              |
| Durability score or mean time to fail MTTF (number of shots after which ball starts to crack/fail) | 34                               | 60                                 | 47                                 | 62                                 |

Compression is measured by applying a 200 pound load to the core and measuring its deflection, in inches. Compression=180-(deflection\*1000).

#### Durability testing of solid cores

Cores were shot at 150 fps in a pneumatic testing machine (PTM).

For each formula mentioned in Table 1, twelve cores were tested. The number of shots after which each core cracked was recorded for each core, and the cracked core was removed from the remainder of the test. The data was reported using a Weibull plot, and the mean time to fail was reported as shown in Table 1. It is reasonable to assume that the durability of a golf ball having a single piece core of this design will also experience a dramatic increase in crack durability based on this improvement to the core.

#### Dual Cores with graphene A only in the outer core.

In this study graphene A was introduced to the outer core in a dual core construction. Dual cores were made by compression molding two outer core halves around an

TABLE 2

| Inner core recipe          |       |
|----------------------------|-------|
| Components                 | % wt  |
| Polybutadiene rubber       | 69.2  |
| Polyisoprene rubber        | 0.0   |
| Zinc diacrylate            | 14.8  |
| Zinc oxide                 | 12.2  |
| Zinc stearate              | 2.1   |
| Peroxide initiator         | 1.0   |
| Zinc pentachlorothiophenol | 0.6   |
| Color                      | 0.1   |
| Barium sulfate             | 0.0   |
| Graphene A                 | 0.0   |
| graphene A masterbatch     | 0.0   |
| Properties                 |       |
| Compression                | 0.220 |

TABLE 3

| Components                                                   | Outer core recipe of dual core        |                                         |                                         |                                         |
|--------------------------------------------------------------|---------------------------------------|-----------------------------------------|-----------------------------------------|-----------------------------------------|
|                                                              | Formula 5<br>(0%<br>Graphene)<br>% wt | Formula 6<br>(0.4%<br>Graphene)<br>% wt | Formula 7<br>(0.8%<br>Graphene)<br>% wt | Formula 8<br>(1.6%<br>Graphene)<br>% wt |
| Polybutadiene                                                | 62.5                                  | 62.3                                    | 62.1                                    | 61.5                                    |
| Zinc Diacrylate                                              | 19.9                                  | 19.8                                    | 19.7                                    | 19.6                                    |
| Zinc Oxide                                                   | 6.3                                   | 6.2                                     | 6.2                                     | 6.2                                     |
| Zinc Stearate                                                | 3.8                                   | 3.7                                     | 3.7                                     | 3.7                                     |
| Peroxide initiator                                           | 0.5                                   | 0.5                                     | 0.5                                     | 0.5                                     |
| Zinc pentachlorothiophenol                                   | 0.6                                   | 0.6                                     | 0.6                                     | 0.6                                     |
| Color                                                        | 0.1                                   | 0.1                                     | 0.1                                     | 0.1                                     |
| Limestone                                                    | 0.0                                   | 0.0                                     | 0.0                                     | 0.0                                     |
| Tungsten                                                     | 0.0                                   | 0.0                                     | 0.0                                     | 0.0                                     |
| Barium sulfate                                               | 6.4                                   | 6.4                                     | 6.4                                     | 6.3                                     |
| Graphene A                                                   | 0.0                                   | 0.4                                     | 0.8                                     | 1.6                                     |
| Graphene A in masterbatch                                    | 0.0                                   | 0.0                                     | 0.0                                     | 0.0                                     |
| Properties of outer core                                     |                                       |                                         |                                         |                                         |
| Compression                                                  | 69.4                                  | 74.3                                    | 74.6                                    | 76.4                                    |
| COR (coefficient of restitution)                             | 0.801                                 | 0.800                                   | 0.795                                   | 0.790                                   |
| Properties of dual core built from inner and outer core      |                                       |                                         |                                         |                                         |
| Compression                                                  | 48.9                                  | 50.9                                    | 52.1                                    | 54.1                                    |
| COR (coefficient of restitution @ 125 fps)                   | 0.796                                 | 0.795                                   | 0.793                                   | 0.790                                   |
| Durability score or mean time to fail                        | 50                                    | 60                                      | 52                                      | 57                                      |
| MTTF (number of shots after which ball starts to crack/fail) |                                       |                                         |                                         |                                         |

Compression is measured by applying a 200 pound load to the core and measuring its deflection, in inches. Compression=180-(deflection\*1000)

#### Durability testing of dual cores

Cores were shot at 175 fps in a pneumatic testing machine (PTM).

For each formula mentioned in Table 3, twelve cores were tested. The number of shots after which each core cracked was recorded for each core, and the cracked core was removed from the remainder of the test. The data was reported using a Weibull plot, and the mean time to fail was reported as shown in Table 3. It is reasonable to assume that the durability of a golf ball having a dual core of this design will also experience a dramatic increase in crack durability based on this improvement to the dual core. It is reasonable to assume that the addition of graphene in the inner core

could provide a durability enhancement to the overall golf ball, but this study only focused on the outer core.

#### Dual cores with Graphene-C in outer core only

In this study Graphene-C (0.01-6%, available from various suppliers such as Cheap Tubes Inc., Ad-Nano Technologies Private Limited, MKnano, XG Sciences Inc., Angstrom Materials Inc., and has an average surface area between 400-800 m<sup>2</sup>/g) was introduced to the outer core in a dual core construction. Dual cores were made by compression molding two outer core halves around an already molded inner core having a diameter of approximately 0.940" and a soft compression of approximately 0.200 inches of deflection under a 200 lb load. Curing of the inner and outer core was done at temperatures ranging between 150-400 F for times ranging from 1-30 minutes. After molding, the dual cores were spherically ground to approximately 1.554" prior to testing.

Tables 4 and 5 give details of recipe of inner and outer cores. Components from these recipes were mixed in an internal mixer. Optionally, additional mixing was done using a two roll mill.

Compression of the outer core is measured by first making a full size core separately, measuring its compression, and then molding two halves around the inner core to complete the dual core. Compression differential describes the difference between the outer core compression (as molded independently) and inner core compression. A higher compression differential is more susceptible to crack durability upon impact.

TABLE 4

| Components                 | Inner core recipe            |      |
|----------------------------|------------------------------|------|
|                            |                              | % wt |
| Polybutadiene rubber       |                              | 69.2 |
| Polyisoprene rubber        |                              | 0.0  |
| Zinc diacrylate            |                              | 14.8 |
| Zinc oxide                 |                              | 12.2 |
| Zinc stearate              |                              | 2.1  |
| Peroxide initiator         |                              | 1.0  |
| Zinc pentachlorothiophenol |                              | 0.6  |
| Color                      |                              | 0.1  |
| Barium sulfate             |                              | 0.0  |
| Graphene-C                 |                              | 0.0  |
| Graphene-C masterbatch     |                              | 0.0  |
| Properties                 |                              |      |
| Compression                | 0.220 inch under 200 lb load |      |

TABLE 5

| Components                 | Outer recipe of dual core               |                                            |                                            |                                            |
|----------------------------|-----------------------------------------|--------------------------------------------|--------------------------------------------|--------------------------------------------|
|                            | Formula 9<br>(0%<br>Graphene C)<br>% wt | Formula 10<br>(0.4%<br>Graphene C)<br>% wt | Formula 11<br>(0.8%<br>Graphene C)<br>% wt | Formula 12<br>(1.6%<br>Graphene C)<br>% wt |
| Polybutadiene              | 62.5                                    | 62.3                                       | 62.0                                       | 61.6                                       |
| Zinc Diacrylate            | 19.9                                    | 19.8                                       | 19.7                                       | 19.6                                       |
| Zinc Oxide                 | 6.3                                     | 6.2                                        | 6.2                                        | 6.2                                        |
| Zinc Stearate              | 3.8                                     | 3.7                                        | 3.7                                        | 3.7                                        |
| Peroxide initiator         | 0.5                                     | 0.5                                        | 0.5                                        | 0.5                                        |
| Zinc pentachlorothiophenol | 0.6                                     | 0.6                                        | 0.6                                        | 0.6                                        |
| Color                      | 0.1                                     | 0.1                                        | 0.1                                        | 0.1                                        |
| Limestone                  | 0.0                                     | 0.0                                        | 0.0                                        | 0.0                                        |
| Tungsten                   | 0.0                                     | 0.0                                        | 0.0                                        | 0.0                                        |
| Barium sulfate             | 6.4                                     | 6.4                                        | 6.4                                        | 6.3                                        |
| Graphene-2                 | 0.0                                     | 0.4                                        | 0.8                                        | 1.6                                        |
| Graphene-2 in masterbatch  | 0.0                                     | 0.0                                        | 0.0                                        | 0.0                                        |

TABLE 5-continued

| Components                                                                                         | Outer recipe of dual core               |                                            |                                            |                                            |
|----------------------------------------------------------------------------------------------------|-----------------------------------------|--------------------------------------------|--------------------------------------------|--------------------------------------------|
|                                                                                                    | Formula 9<br>(0%<br>Graphene C)<br>% wt | Formula 10<br>(0.4%<br>Graphene C)<br>% wt | Formula 11<br>(0.8%<br>Graphene C)<br>% wt | Formula 12<br>(1.6%<br>Graphene C)<br>% wt |
|                                                                                                    | Properties of outer core                |                                            |                                            |                                            |
| Compression                                                                                        | 67.0                                    | 69.1                                       | 68.8                                       | 70.8                                       |
| COR (coefficient of restitution)                                                                   | 0.801                                   | 0.798                                      | 0.795                                      | 0.791                                      |
| Core Stiffness/Flexural Modulus in MPa (measured on dog bone shape cured core)                     | 97.1                                    | 91.3                                       | 94.6                                       | 81.9                                       |
| Tensile modulus of the core in MPa (measured on a dog bone shaped cured core)                      | 8.5                                     | 9.7                                        | 9.6                                        | 8.3                                        |
| Properties of dual core built from inner and outer core                                            |                                         |                                            |                                            |                                            |
| Compression                                                                                        | 45.0                                    | 48.9                                       | 48.6                                       | 50.4                                       |
| COR (coefficient of restitution @ 125 fps)                                                         | 0.795                                   | 0.794                                      | 0.793                                      | 0.789                                      |
| Durability score or mean time to fail MTTF (number of shots after which ball starts to crack/fail) | 33                                      | 67                                         | 78                                         | 99                                         |

Compression is measured by applying a 200 pound load to the core and measuring its deflection, in inches. Compression=180-(deflection\*1000).

#### Durability testing of dual cores

Cores were shot at 175 fps in a pneumatic testing machine (PTM).

For each formula mentioned in Table 5, twelve cores were tested. The number of shots after which each core cracked was recorded for each core, and the cracked core was removed from the remainder of the test. The data was reported using a Weibull plot, and the mean time to fail was reported as shown in Table 5. Testing was stopped after 100 shots. It is reasonable to assume that the durability of a golf ball having a dual core of this design will also experience a dramatic increase in crack durability based on this improvement to the dual core. It is reasonable to assume that the addition of graphene in the inner core could provide a durability enhancement to the overall golf ball, but this study only focused on the outer core.

Dual cores with graphene A in the inner core and the outer core.

In this study graphene A was introduced to the inner and outer core in a dual core construction. Table 6 gives details of recipe of inner and outer cores of these dual cores. Components from these recipes were mixed in an internal mixer. Optionally, additional mixing was done using a two roll mill. Dual cores were made by compression molding two outer core halves around an already molded inner core having a diameter of approximately 0.940" and a soft compression of approximately 0.200 inches of deflection under a 200 lb load. Curing of the inner and outer core was done at temperatures ranging between 150-400 F for times ranging from 1-30 minutes. After molding, the dual cores were spherically ground to approximately 1.554" prior to testing.

Compression of the outer core was measured by first making a full size core separately, measuring its compression, and then molding two halves around the inner core to complete the dual core.

TABLE 6

Dual core recipes with graphene A in the inner core and the outer core

| Components                 | Formula 13-<br>inner core | Formula 14-<br>inner core | Formula 15-<br>inner core | Formula 16-<br>inner core |
|----------------------------|---------------------------|---------------------------|---------------------------|---------------------------|
|                            | % wt                      | % wt                      | % wt                      | % wt                      |
| Polybutadiene              | 69.2                      | 69.2                      | 69.1                      | 68.9                      |
| Zinc Diacrylate            | 14.8                      | 14.8                      | 14.7                      | 14.7                      |
| Zinc Oxide                 | 12.3                      | 12.3                      | 12.2                      | 12.2                      |
| Zinc Stearate              | 2.1                       | 2.1                       | 2.1                       | 2.1                       |
| Peroxide initiator         | 1.0                       | 1.0                       | 1.0                       | 1.0                       |
| Zinc pentachlorothiophenol | 0.6                       | 0.6                       | 0.6                       | 0.6                       |
| Color                      | 0.0                       | 0.0                       | 0.0                       | 0.0                       |
| Limestone                  | 0.0                       | 0.0                       | 0.0                       | 0.0                       |
| Tungsten                   | 0.0                       | 0.0                       | 0.0                       | 0.0                       |

TABLE 6-continued

| Dual core recipes with graphene A in the inner core and the outer core                                      |                                   |                                   |                                   |                                   |
|-------------------------------------------------------------------------------------------------------------|-----------------------------------|-----------------------------------|-----------------------------------|-----------------------------------|
| Barium sulfate                                                                                              | 0.0                               | 0.0                               | 0.0                               | 0.0                               |
| Graphene A                                                                                                  | 0.0                               | 0.0                               | 0.2                               | 0.4                               |
| Properties of inner core                                                                                    |                                   |                                   |                                   |                                   |
| Compression                                                                                                 | 0.221                             | 0.221                             | 0.219                             | 0.217                             |
| Properties of outer core                                                                                    |                                   |                                   |                                   |                                   |
| Components                                                                                                  | Formula 13-<br>outer core<br>% wt | Formula 14-<br>outer core<br>% wt | Formula 15-<br>outer core<br>% wt | Formula 16-<br>outer core<br>% wt |
| Polybutadiene                                                                                               | 62.5                              | 62.3                              | 62.3                              | 62.3                              |
| Zinc Diacrylate                                                                                             | 19.9                              | 19.8                              | 19.8                              | 19.8                              |
| Zinc Oxide                                                                                                  | 6.2                               | 6.2                               | 6.2                               | 6.2                               |
| Zinc Stearate                                                                                               | 3.7                               | 3.7                               | 3.7                               | 3.7                               |
| Peroxide initiator                                                                                          | 0.5                               | 0.5                               | 0.5                               | 0.5                               |
| Zinc pentachlorothiophenol                                                                                  | 0.6                               | 0.6                               | 0.6                               | 0.6                               |
| Color                                                                                                       | 0.1                               | 0.0                               | 0.0                               | 0.0                               |
| Limestone                                                                                                   | 0.0                               | 0.0                               | 0.0                               | 0.0                               |
| Tungsten                                                                                                    | 0.0                               | 0.0                               | 0.0                               | 0.0                               |
| Barium sulfate                                                                                              | 6.5                               | 6.5                               | 6.5                               | 6.5                               |
| Graphene A                                                                                                  | 0.0                               | 0.4                               | 0.4                               | 0.4                               |
| Properties of dual core built from inner and outer core                                                     |                                   |                                   |                                   |                                   |
| Compression                                                                                                 | 67.8                              | 67.6                              | 67.6                              | 67.6                              |
| COR (coefficient of<br>restitution @ 125 fps)                                                               | 0.800                             | 0.796                             | 0.796                             | 0.796                             |
| Properties of dual core built from inner and outer core                                                     |                                   |                                   |                                   |                                   |
| Compression                                                                                                 | 47.3                              | 48.1                              | 49.0                              | 48.3                              |
| COR (coefficient of<br>restitution @ 125 fps)                                                               | 0.795                             | 0.793                             | 0.793                             | 0.792                             |
| Durability score or mean time<br>to fail MTTF (number of shots<br>after which ball starts to<br>crack/fail) | 29                                | 24                                | 33                                | 40                                |

Compression is measured by applying a 200 pound load to the core and measuring its deflection, in inches. Compression=180-(deflection\*1000).

For each formula mentioned in Table 6, twelve cores were tested. The number of shots after which each core cracked was recorded for each core, and the cracked core was removed from the remainder of the test. The data was reported using a Weibull plot, and the mean time to fail was reported as shown in Table 6. The best durability was observed for balls which had graphene in inner and outer cores. It is reasonable to assume that the durability of a golf ball having a dual core of this design will also experience a dramatic increase in crack durability based on this improvement to the dual core. It is reasonable to assume that the addition of graphene in the inner core could provide a durability enhancement to the overall golf ball, but this study only focused on the outer core.

#### Dual Cores With Graphene B In The Outer Core Only

In this study Graphene-B was introduced to the outer core in a dual core construction. Dual cores were made by compression molding two outer core halves around an already molded inner core having a diameter of approximately 0.940" and a soft compression of approximately 0.200 inches of deflection under a 200 lb load. Curing of the inner and outer core was done at temperatures ranging between 150-400 F for times ranging from 1-30 minutes. After molding, the dual cores were spherically ground to approximately 1.554" prior to testing.

Compression of the outer core is measured by first making a full size core separately, measuring its compression, and then molding two halves around the inner core to complete the dual core. Compression differential describes the difference between the outer core compression (as molded inde-

pendently) and inner core compression. A higher compression differential is more susceptible to crack durability upon impact.

TABLE 7

| Inner Core Recipe          |                              |
|----------------------------|------------------------------|
| Components                 | % wt                         |
| Polybutadiene rubber       | 69.2                         |
| Polyisoprene rubber        | 0.0                          |
| Zinc diacrylate            | 14.8                         |
| Zinc oxide                 | 12.2                         |
| Zinc stearate              | 2.1                          |
| Peroxide initiator         | 1.0                          |
| Zinc pentachlorothiophenol | 0.6                          |
| Color                      | 0.1                          |
| Barium sulfate             | 0.0                          |
| Graphene-B                 | 0.0                          |
| Graphene-B masterbatch     | 0.0                          |
| Properties                 |                              |
| Compression                | 0.223 inch under 200 lb load |

Novelty of this process: Durability of the dual core with a high compression differential is greatly enhanced by incorporation of graphene in inner and outer core. The graphene reinforcement to the inner and outer core helps resist the high stresses experienced by the core when struck at high club speeds. Addition of graphene to the core recipe is very simple and it can be dispersed into the polybutadiene mixture during two roll milling process. Due to high thermal conductivity of graphene, overall thermal conductivity of cores can be increased with incorporation of graphene. With higher thermal conductivity of graphene reinforced cores,

curing cycles can be made shorter. Shorter curing cycles can lead to higher output in production. Optionally, graphene can be introduced as a masterbatch in polybutadiene or polyisoprene, making its dispersion into polybutadiene rubber much easier and dust free.

#### Dual Core

As our experiment has shown, incorporating graphene into the inner and outer core recipe reinforces the strength of the outer core and provides greater crack durability protection in the design of a dual core golf ball, which is more susceptible to crack durability failures if the outer core is much firmer than the soft inner core.

In general, this is applicable when the inner core is softer than the outer core. More specifically, when the inner core has more than 0.200" deflection under a 200 lb load, and the dual core is 40 compression or greater.

This is particularly crucial if the ball is a 4-piece construction with a single mantle layer with thickness less than 0.050", or more specifically thinner than 0.040", with being the target in this study.

FIGS. 1, 3, 4 and 5 illustrate a five piece golf ball 10 comprising an inner core 12a, an outer core 12b, an inner mantle 14a, an outer mantle 14b, and a cover 16, wherein the cover layer 16 is composed of a polyurethane and ionomer hybrid formed by compounding or dry blending acid functional polyurethane and ionomer. The inner core 12a comprises polybutadiene mixture comprising 0.4 to 2.5 weight percent of a graphene.

FIG. 5A illustrates a five piece golf ball 10 comprising an inner core 12a, an intermediate core 12b, an outer core 12c, a mantle 14, and a cover 16, wherein the cover layer 16 is composed of a polyurethane and ionomer hybrid formed by compounding or dry blending acid functional polyurethane and ionomer. The intermediate core 12b comprises polybutadiene mixture comprising 0.4 to 2.5 weight percent of a graphene.

FIGS. 8 and 9 illustrate a six piece golf ball 10 comprising an inner core 12a, an intermediate core 12b, an outer core 12c, an inner mantle 14a, an outer mantle 14b, and a cover 16, wherein the cover layer 16 is composed of a polyurethane and ionomer hybrid formed by compounding or dry blending acid functional polyurethane and ionomer. The inner core 12a comprises polybutadiene mixture comprising 0.4 to 2.5 weight percent of a graphene.

FIG. 10 illustrates a four piece golf ball comprising a dual core, a boundary layer and a cover composed of a polyurethane and ionomer hybrid formed by compounding or dry blending acid functional polyurethane and ionomer. The outer core comprises polybutadiene mixture comprising 0.4 to 2.5 weight percent of a graphene.

FIG. 11 illustrates a three piece golf ball comprising a core, a boundary layer and a cover. The core comprises polybutadiene mixture comprising 0.4 to 2.5 weight percent of a graphene.

FIGS. 12 and 13 illustrate a two piece golf ball 20 with a core 25 and a cover 30. The core comprises polybutadiene mixture comprising 0.4 to 2.5 weight percent of a graphene.

FIGS. 14 and 15 illustrate a three-piece golf ball 5 comprising a core 10, a mantle layer 14 and a cover 16 with dimples 18, wherein the core comprises 0.4 to 2.5 weight percent of a graphene.

FIG. 16 illustrates a dual core three piece golf ball 35 comprising an inner core and outer core 32 and a cover 34, wherein the core comprises 0.4 to 2.5 weight percent of a graphene.

FIG. 17 illustrates a three piece golf ball 45 comprising a core 40, a mantle layer 42 and a cover 44, wherein the core comprises 0.4 to 2.5 weight percent of a graphene.

FIG. 18 illustrates a dual core four piece golf ball 55 comprising an inner core 50, an outer core 52, a mantle layer 54 and a cover 56, wherein the core comprises 0.4 to 2.5 weight percent of a graphene.

FIG. 19 illustrates a four piece golf ball 65 comprising a core 60, an inner mantle 62, an outer mantle 64 and a cover 66, wherein the core comprises 0.4 to 2.5 weight percent of a graphene.

The mantle component is preferably composed of the inner mantle layer and the outer mantle layer. The mantle component preferably has a thickness ranging from 0.05 inch to 0.15 inch, and more preferably from 0.06 inch to 0.08 inch. The outer mantle layer is preferably composed of a blend of ionomer materials. One preferred embodiment comprises SURLYN 9150 material, SURLYN 8940 material, a SURLYN AD1022 material, and a masterbatch. The SURLYN 9150 material is preferably present in an amount ranging from 20 to 45 weight percent of the cover, and more preferably 30 to 40 weight percent. The SURLYN 8945 is preferably present in an amount ranging from 15 to 35 weight percent of the cover, more preferably 20 to 30 weight percent, and most preferably 26 weight percent. The SURLYN 9945 is preferably present in an amount ranging from 30 to 50 weight percent of the cover, more preferably 35 to 45 weight percent, and most preferably 41 weight percent. The SURLYN 8940 is preferably present in an amount ranging from 5 to 15 weight percent of the cover, more preferably 7 to 12 weight percent, and most preferably 10 weight percent.

SURLYN 8320, from DuPont, is a very-low modulus ethylene/methacrylic acid copolymer with partial neutralization of the acid groups with sodium ions. SURLYN 8945, also from DuPont, is a high acid ethylene/methacrylic acid copolymer with partial neutralization of the acid groups with sodium ions. SURLYN 9945, also from DuPont, is a high acid ethylene/methacrylic acid copolymer with partial neutralization of the acid groups with zinc ions. SURLYN 8940, also from DuPont, is an ethylene/methacrylic acid copolymer with partial neutralization of the acid groups with sodium ions.

The inner mantle layer is preferably composed of a blend of ionomers, preferably comprising a terpolymer and at least two high acid (greater than 18 weight percent) ionomers neutralized with sodium, zinc, magnesium, or other metal ions. The material for the inner mantle layer preferably has a Shore D plaque hardness ranging preferably from 35 to 77, more preferably from 36 to 44, a most preferably approximately 40. The thickness of the outer mantle layer preferably ranges from 0.025 inch to 0.050 inch, and is more preferably approximately 0.037 inch. The mass of an insert including the dual core and the inner mantle layer preferably ranges from 32 grams to 40 grams, more preferably from 34 to 38 grams, and is most preferably approximately 36 grams. The inner mantle layer is alternatively composed of a HPF material available from DuPont. Alternatively, the inner mantle layer 14b is composed of a material such as disclosed in Kennedy, III et al., U.S. Pat. No. 7,361,101 for a Golf Ball And Thermoplastic Material, which is hereby incorporated by reference in its entirety.

The outer mantle layer is preferably composed of a blend of ionomers, preferably comprising at least two high acid (greater than 18 weight percent) ionomers neutralized with sodium, zinc, or other metal ions. The blend of ionomers also preferably includes a masterbatch. The material of the

outer mantle layer preferably has a Shore D plaque hardness ranging preferably from 55 to 75, more preferably from 65 to 71, and most preferably approximately 67. The thickness of the outer mantle layer preferably ranges from 0.025 inch to 0.040 inch, and is more preferably approximately 0.030 inch. The mass of the entire insert including the core, the inner mantle layer and the outer mantle layer preferably ranges from 38 grams to 43 grams, more preferably from 39 to 41 grams, and is most preferably approximately 41 grams.

In an alternative embodiment, the inner mantle layer is preferably composed of a blend of ionomers, preferably comprising at least two high acid (greater than 18 weight percent) ionomers neutralized with sodium, zinc, or other metal ions. The blend of ionomers also preferably includes a masterbatch. In this embodiment, the material of the inner mantle layer has a Shore D plaque hardness ranging preferably from 55 to 75, more preferably from 65 to 71, and most preferably approximately 67. The thickness of the outer mantle layer preferably ranges from 0.025 inch to 0.040 inch, and is more preferably approximately 0.030 inch. Also in this embodiment, the outer mantle layer **14b** is composed of a blend of ionomers, preferably comprising a terpolymer and at least two high acid (greater than 18 weight percent) ionomers neutralized with sodium, zinc, magnesium, or other metal ions. In this embodiment, the material for the outer mantle layer **14b** preferably has a Shore D plaque hardness ranging preferably from 35 to 77, more preferably from 36 to 44, a most preferably approximately 40. The thickness of the outer mantle layer preferably ranges from 0.025 inch to 0.100 inch, and more preferably ranges from 0.070 inch to 0.090 inch.

In yet another embodiment wherein the inner mantle layer is thicker than the outer mantle layer and the outer mantle layer is harder than the inner mantle layer, the inner mantle layer is composed of a blend of ionomers, preferably comprising a terpolymer and at least two high acid (greater than 18 weight percent) ionomers neutralized with sodium, zinc, magnesium, or other metal ions. In this embodiment, the material for the inner mantle layer has a Shore D plaque hardness ranging preferably from 30 to 77, more preferably from 30 to 50, and most preferably approximately 40. In this embodiment, the material for the outer mantle layer has a Shore D plaque hardness ranging preferably from 40 to 77, more preferably from 50 to 71, and most preferably approximately 67. In this embodiment, the thickness of the inner mantle layer preferably ranges from 0.030 inch to 0.090 inch, and the thickness of the outer mantle layer ranges from 0.025 inch to 0.070 inch.

Preferably the inner core has a diameter ranging from 0.75 inch to 1.20 inches, more preferably from 0.85 inch to 1.05 inch, and most preferably approximately 0.95 inch. Preferably the inner core **12a** has a Shore D hardness ranging from 20 to 50, more preferably from 25 to 40, and most preferably approximately 35. Preferably the inner core has a mass ranging from 5 grams to 15 grams, 7 grams to 10 grams and most preferably approximately 8 grams.

Preferably the outer core has a diameter ranging from 1.25 inch to 1.55 inches, more preferably from 1.40 inch to 1.5 inch, and most preferably approximately 1.5 inch. Preferably the outer core has a Shore D surface hardness ranging from 40 to 65, more preferably from 50 to 60, and most preferably approximately 56. Preferably the outer core is formed from a polybutadiene, zinc diacrylate, zinc oxide, zinc stearate, a peptizer and peroxide. Preferably the combined inner core and outer core have a mass ranging from 25 grams to 35 grams, 30 grams to 34 grams and most preferably approximately 32 grams.

Preferably the inner core has a deflection of at least 0.230 inch under a load of 220 pounds, and the core has a deflection of at least 0.080 inch under a load of 200 pounds. As shown in FIGS. 6 and 7, a mass **50** is loaded onto an inner core and a core. As shown in FIGS. 6 and 7, the mass is 100 kilograms, approximately 220 pounds. Under a load of 100 kilograms, the inner core preferably has a deflection from 0.230 inch to 1 inch. Under a load of 100 kilograms, preferably the core has a deflection of 0.08 inch to 0.150 inch. Alternatively, the load is 200 pounds (approximately 90 kilograms), and the deflection of the core **12** is at least 0.080 inch. Further, a compressive deformation from a beginning load of 10 kilograms to an ending load of 130 kilograms for the inner core ranges from 4 millimeters to 7 millimeters and more preferably from 5 millimeters to 6.5 millimeters. The dual core deflection differential allows for low spin off the tee to provide greater distance, and high spin on approach shots.

In an alternative embodiment of the golf ball shown in FIG. 5A, the golf ball **10** comprises an inner core **12a**, an intermediate core **12b**, an outer core **12b**, a mantle **14** and a cover **16**. The golf ball **10** preferably has a diameter of at least 1.68 inches, a mass ranging from 45 grams to 47 grams, a COR of at least 0.79, a deformation under a 100 kilogram loading of at least 0.07 mm.

In one embodiment, the golf ball comprises a core, a mantle layer and a cover layer. The core comprises an inner core sphere, an intermediate core layer and an outer core layer. The intermediate core layer is composed of a highly neutralized ionomer and has a Shore D hardness less than 40. The outer core layer is composed of a highly neutralized ionomer and has a Shore D hardness less than 45. A thickness of the intermediate core layer is greater than a thickness of the outer core layer. The mantle layer is disposed over the core, comprises an ionomer material and has a Shore D hardness greater than 55. The cover layer is disposed over the mantle layer comprises a thermoplastic polyurethane material and has a Shore A hardness less than 100. The golf ball has a diameter of at least 1.68 inches. The mantle layer is harder than the outer core layer, the outer core layer is harder than the intermediate core layer, the intermediate core layer is harder than the inner core sphere, and the cover layer is softer than the mantle layer.

In another embodiment, shown in FIGS. 8 and 9, the golf ball **10** has a multi-layer core and multi-layer mantle. The golf ball includes a core, a mantle component and a cover layer. The core comprises an inner core sphere, an intermediate core layer and an outer core layer. The inner core sphere comprises a TPEE material and has a diameter ranging from 0.875 inch to 1.4 inches. The intermediate core layer is composed of a highly neutralized ionomer and has a Shore D hardness less than 40. The outer core layer is composed of a highly neutralized ionomer and has a Shore D hardness less than 45. A thickness of the intermediate core layer is greater than a thickness of the outer core layer **12c**. The inner mantle layer is disposed over the core, comprises an ionomer material and has a Shore D hardness greater than 55. The outer mantle layer is disposed over the inner mantle layer, comprises an ionomer material and has a Shore D hardness greater than 60. The cover layer is disposed over the mantle component, comprises a thermoplastic polyurethane material and has a Shore A hardness less than 100. The golf ball has a diameter of at least 1.68 inches. The outer mantle layer is harder than the inner mantle layer, the inner mantle layer is harder than the outer core layer, the outer core layer is harder than the intermediate core layer, the intermediate core layer is harder than the inner core sphere, and the cover layer is softer than the mantle layer.

intermediate core layer is harder than the inner core sphere, and the cover layer is softer than the outer mantle layer.

In a particularly preferred embodiment of the invention, the golf ball preferably has an aerodynamic pattern such as disclosed in Simonds et al., U.S. Pat. No. 7,419,443 for a Low Volume Cover For A Golf Ball, which is hereby incorporated by reference in its entirety. Alternatively, the golf ball has an aerodynamic pattern such as disclosed in Simonds et al., U.S. Pat. No. 7,338,392 for An Aerodynamic Surface Geometry For A Golf Ball, which is hereby incorporated by reference in its entirety.

Various aspects of the present invention golf balls have been described in terms of certain tests or measuring procedures. These are described in greater detail as follows.

As used herein, "Shore D hardness" of the golf ball layers is measured generally in accordance with ASTM D-2240 type D, except the measurements may be made on the curved surface of a component of the golf ball, rather than on a plaque. If measured on the ball, the measurement will indicate that the measurement was made on the ball. In referring to a hardness of a material of a layer of the golf ball, the measurement will be made on a plaque in accordance with ASTM D-2240. Furthermore, the Shore D hardness of the cover is measured while the cover remains over the mantles and cores. When a hardness measurement is made on the golf ball, the Shore D hardness is preferably measured at a land area of the cover.

As used herein, "Shore A hardness" of a cover is measured generally in accordance with ASTM D-2240 type A, except the measurements may be made on the curved surface of a component of the golf ball, rather than on a plaque. If measured on the ball, the measurement will indicate that the measurement was made on the ball. In referring to a hardness of a material of a layer of the golf ball, the measurement will be made on a plaque in accordance with ASTM D-2240. Furthermore, the Shore A hardness of the cover is measured while the cover remains over the mantles and cores. When a hardness measurement is made on the golf ball, Shore A hardness is preferably measured at a land area of the cover.

The resilience or coefficient of restitution (COR) of a golf ball is the constant "e," which is the ratio of the relative velocity of an elastic sphere after direct impact to that before impact. As a result, the COR ("e") can vary from 0 to 1, with 1 being equivalent to a perfectly or completely elastic collision and 0 being equivalent to a perfectly or completely inelastic collision.

COR, along with additional factors such as club head speed, club head mass, ball weight, ball size and density, spin rate, angle of trajectory and surface configuration as well as environmental conditions (e.g. temperature, moisture, atmospheric pressure, wind, etc.) generally determine the distance a ball will travel when hit. Along this line, the distance a golf ball will travel under controlled environmental conditions is a function of the speed and mass of the club and size, density and resilience (COR) of the ball and other factors. The initial velocity of the club, the mass of the club and the angle of the ball's departure are essentially provided by the golfer upon striking. Since club head speed, club head mass, the angle of trajectory and environmental conditions are not determinants controllable by golf ball producers and the ball size and weight are set by the U.S.G.A., these are not factors of concern among golf ball manufacturers. The factors or determinants of interest with respect to improved distance are generally the COR and the surface configuration of the ball.

The coefficient of restitution is the ratio of the outgoing velocity to the incoming velocity. In the examples of this application, the coefficient of restitution of a golf ball was measured by propelling a ball horizontally at a speed of 125 $\pm$ 5 feet per second (fps) and corrected to 125 fps against a generally vertical, hard, flat steel plate and measuring the ball's incoming and outgoing velocity electronically. Speeds were measured with a pair of ballistic screens, which provide a timing pulse when an object passes through them. The screens were separated by 36 inches and are located 25.25 inches and 61.25 inches from the rebound wall. The ball speed was measured by timing the pulses from screen 1 to screen 2 on the way into the rebound wall (as the average speed of the ball over 36 inches), and then the exit speed was timed from screen 2 to screen 1 over the same distance. The rebound wall was tilted 2 degrees from a vertical plane to allow the ball to rebound slightly downward in order to miss the edge of the cannon that fired it. The rebound wall is solid steel.

As indicated above, the incoming speed should be 125  $\pm$  5 fps but corrected to 125 fps. The correlation between COR and forward or incoming speed has been studied and a correction has been made over the  $\pm$ 5 fps range so that the COR is reported as if the ball had an incoming speed of exactly 125.0 fps.

The measurements for deflection, compression, hardness, and the like are preferably performed on a finished golf ball as opposed to performing the measurement on each layer during manufacturing.

Preferably, in a five layer golf ball comprising an inner core, an outer core, an inner mantle layer, an outer mantle layer and a cover, the hardness/compression of layers involve an inner core with the greatest deflection (lowest hardness), an outer core (combined with the inner core) with a deflection less than the inner core, an inner mantle layer with a hardness less than the hardness of the combined outer core and inner core, an outer mantle layer with the hardness layer of the golf ball, and a cover with a hardness less than the hardness of the outer mantle layer. These measurements are preferably made on a finished golf ball that has been torn down for the measurements.

Preferably the inner mantle layer is thicker than the outer mantle layer or the cover layer. The dual core and dual mantle golf ball creates an optimized velocity-initial velocity ratio (Vi/IV), and allows for spin manipulation. The dual core provides for increased core compression differential resulting in a high spin for short game shots and a low spin for driver shots. A discussion of the USGA initial velocity test is disclosed in Yagley et al., U.S. Pat. No. 6,595,872 for a Golf Ball With High Coefficient Of Restitution, which is hereby incorporated by reference in its entirety. Another example is Bartels et al., U.S. Pat. No. 6,648,775 for a Golf Ball With High Coefficient Of Restitution, which is hereby incorporated by reference in its entirety.

Alternatively, the cover 16 is composed of a thermoplastic polyurethane/polyurea material. One example is disclosed in U.S. Pat. No. 7,367,903 for a Golf Ball, which is hereby incorporated by reference in its entirety. Another example is Melanson, U.S. Pat. No. 7,641,841, which is hereby incorporated by reference in its entirety. Another example is Melanson et al., U.S. Pat. No. 7,842,211, which is hereby incorporated by reference in its entirety. Another example is Matroni et al., U.S. Pat. No. 7,867,111, which is hereby incorporated by reference in its entirety. Another example is Dewanjee et al., U.S. Pat. No. 7,785,522, which is hereby incorporated by reference in its entirety.

## 17

Bartels, U.S. Pat. No. 9,278,260, for a Low Compression Three-Piece Golf Ball With An Aerodynamic Drag Rise At High Speeds, is hereby incorporated by reference in its entirety.

Chavan et al, U.S. Pat. No. 9,789,366, for a Graphene Core For A Golf Ball, is hereby incorporated by reference in its entirety.

Chavan et al, U.S. patent application Ser. No. 15/705011, filed on Sep. 14, 2017, for a Graphene Core For A Golf Ball, is hereby incorporated by reference in its entirety.

Chavan et al, U.S. patent application Ser. No. 15/729,231, filed on Oct. 10, 2017, for a Graphene And Nanotube Reinforced Golf Ball, is hereby incorporated by reference in its entirety.

Brown, U.S. patent application Ser. No. 15/683,398, filed on Aug. 22, 2017, for a Golf Ball With Improved Durability, is hereby incorporated by reference in its entirety.

Crast et al., U.S. Pat. No. 6,632,877, for a Dual Curable Coating, is hereby incorporated by reference in its entirety.

Skrabski et al., U.S. Pat. No. 6,544,337, for a Golf ball Painting System, is hereby incorporated by reference in its entirety.

Reyes et al., U.S. Pat. No. 6,348,011, for a Texture Coating For A Golf Club, is hereby incorporated by reference in its entirety.

Crast et al., U.S. Pat. No. 6,365,679, for a Two component polyurethane clear coat for golf balls, is hereby incorporated by reference in its entirety.

Crast et al., U.S. Pat. No. 6,165,564, for a UV Clearable Clear Coat For Golf Balls, is hereby incorporated by reference in its entirety.

Skrabski et al., U.S. Pat. No. 6,319,563, for a Golf ball Painting Method, is hereby incorporated by reference in its entirety.

Matroni et al., U.S. Pat. No. 7,485,052, for a Golf Ball, is hereby incorporated by reference in its entirety.

Galloway Sr., U.S. Pat. No. 8,197,355, for an Iron-type golf club head with chamfered leading edge, is hereby incorporated by reference in its entirety.

Reyes et al., U.S. Pat. No. 6,435,980, for a Face Coating For A Golf Club Head, is hereby incorporated by reference in its entirety.

From the foregoing it is believed that those skilled in the pertinent art will recognize the meritorious advancement of this invention and will readily understand that while the present invention has been described in association with a preferred embodiment thereof, and other embodiments illustrated in the accompanying drawings, numerous changes, modifications and substitutions of equivalents may be made therein without departing from the spirit and scope of this invention which is intended to be unlimited by the foregoing except as may appear in the following appended claims. Therefore, the embodiments of the invention in which an exclusive property or privilege is claimed are defined in the following appended claims.

I claim as my invention the following:

1. A golf ball comprising:

a center core;

a mantle layer; and

a cover layer disposed over the mantle layer;

wherein at least one of the cover layer or the mantle layer comprises a maleic anhydride functional polymer and an acid functional polyurethane and ionomer hybrid material made by compounding or dry blending an acid functional polyurethane and an ionomer, wherein the acid functional polyurethane and ionomer hybrid mate-

## 18

rial is formed by reacting an isocyanate functional polymer with molecules that have both hydroxyl and acid functionalities;

wherein the acid functional polyurethane and ionomer hybrid material is neutralized with titanium dioxide.

2. The golf ball according to claim 1 further comprising: an outer core disposed over the center core; an inner mantle layer disposed over the outer core, the inner mantle layer having a thickness ranging from 0.025 inch to 0.100 inch, the inner mantle layer composed of an ionomer material, the inner mantle layer material having a plaque Shore D hardness ranging from 25 to 68;

wherein the mantle layer is disposed over the inner mantle layer, the mantle layer having a thickness ranging from 0.025 inch to 0.100 inch;

and

wherein the cover layer is disposed over the mantle layer, the cover layer has a thickness ranging from 0.025 inch to 0.055 inch;

wherein the cover layer has a lower Shore D hardness than the mantle layer, the mantle layer has a higher Shore D hardness than the inner mantle layer, the outer core has a higher Shore D hardness than the inner mantle layer and the center core.

3. The golf ball according to claim 1 further comprising: an outer core disposed over the center core;

an inner mantle layer disposed over the outer core, the inner mantle layer having a thickness ranging from 0.025 inch to 0.100 inch, the inner mantle layer composed of an ionomer material, the inner mantle layer material having a plaque Shore D hardness ranging from 36 to 44;

wherein the mantle layer is disposed over the inner mantle layer, the mantle layer having a thickness ranging from 0.025 inch to 0.100 inch, the mantle layer composed of an ionomer material, the mantle layer material having a plaque Shore D hardness ranging from 50 to 71; and wherein the cover layer is disposed over the mantle layer, the cover layer having a thickness ranging from 0.025 inch to 0.040 inch;

wherein the cover layer has a lower Shore D hardness than the mantle layer, the mantle layer has a higher Shore D hardness than the inner mantle layer, the outer core has a higher Shore D hardness than the inner mantle layer and the center core.

4. The golf ball according to claim 1 further comprising: an inner mantle layer disposed over the center core, the inner mantle layer having a thickness ranging from 0.030 inch to 0.050 inch, the inner mantle layer material having a plaque Shore D hardness ranging from 30 to 40, the inner mantle layer composed of an ionomer material;

a first center mantle layer disposed over the inner mantle layer, the first center mantle layer having a thickness ranging from 0.030 inch to 0.050 inch, the first center mantle layer material having a plaque Shore D hardness ranging from 40 to 55, the first center mantle layer composed of a fully neutralized polymer material;

a second center mantle layer disposed over the second center mantle layer, the second center mantle layer having a thickness ranging from 0.030 inch to 0.050 inch, the second center mantle layer material having a plaque Shore D hardness ranging from 45 to 55, the second center mantle layer composed of a fully neutralized polymer material;

19

wherein the mantle layer is disposed over the second center mantle layer, the mantle layer having a thickness ranging from 0.030 inch to 0.050 inch, the mantle layer composed of a blend of ionomers, the mantle layer material having a plaque Shore D hardness ranging from 60 to 75; and

wherein the cover layer is disposed over the mantle layer, the cover layer having a thickness ranging from 0.025 inch to 0.040 inch.

5. A golf ball comprising:

a dual core comprising an inner core and an outer disposed over the inner core;

a mantle layer disposed over the inner core; and

a cover layer disposed over the mantle layer;

wherein at least one of the cover layer or the mantle layer comprises a maleic anhydride functional polymer and an acid functional polyurethane and ionomer hybrid material made by compounding or dry blending an acid functional polyurethane and an ionomer, wherein the acid functional polyurethane and ionomer hybrid material is formed by reacting an isocyanate functional polymer with molecules that have both hydroxyl and acid functionalities;

wherein the acid functional polyurethane and ionomer hybrid material is neutralized with titanium dioxide.

20

6. The golf ball according to claim 5 wherein the dual core has a diameter ranging from 1.4 inches to 1.6 inches.

7. The golf ball according to claim 5 wherein the outer core comprises polybutadiene and a graphene material.

5 8. The golf ball according to claim 5 wherein the inner core has a deflection under a load of 100 kilogram of at least 0.18 inch.

9. A golf ball comprising:  
a core;

10 an inner mantle layer disposed over the core;  
an outer mantle layer disposed over the inner mantle layer; and

a cover layer disposed over the outer mantle layer;  
wherein at least one of the cover layer, the inner mantle

15 layer or the outer mantle layer comprises a maleic anhydride functional polymer and an acid functional polyurethane and ionomer hybrid material made by compounding or dry blending an acid functional polyurethane and an ionomer, wherein the acid functional polyurethane and ionomer hybrid material is formed by reacting an isocyanate functional polymer with molecules that have both hydroxyl and acid functionalities;  
wherein the acid functional polyurethane and ionomer

20 hybrid material is neutralized with titanium dioxide.

\* \* \* \* \*